

# UNITED STATES PATENT OFFICE.

ALVAH W. CLEMENT, OF CLEVELAND, OHIO, ASSIGNOR TO THE CLEVELAND BRASS MANUFACTURING COMPANY, OF CLEVELAND, OHIO, A CORPORATION OF OHIO.

## ACID-RESISTING ALLOY.

1,375,081.

Specification of Letters Patent. Patented Apr. 19, 1921.

Continuation of application Serial No. 182,912, filed July 26, 1917. This application filed July 27, 1918. Serial No. 246,990.

To all whom it may concern:

Be it known that I, ALVAH W. CLEMENT, a citizen of the United States, residing at Cleveland, in the county of Cuyahoga and State of Ohio, have invented a certain new and useful Improvement in Acid-Resisting Alloys, (C,) of which the following is a full, clear, and exact description.

This application is a continuation of my application, Serial Number 182,912, filed July 26, 1917.

The object of this invention is to produce an alloy which is resistant to the action of acids, among which most prominently may be mentioned sulfuric, nitric, and hydrochloric.

In speaking of this alloy as resistant to acids, it is not intended to go so far as to say that it is resistant to all laboratory tests that might be made with these acids, but practice has demonstrated that in commercial use it is resistant and admirably fulfills its function.

In those industries which require that acids be pumped and conducted from one receptacle or place to another, the only practical conductors which are at present used are made of porcelain or some similar material having inferior physical properties, being brittle and substantially unmachinable. These porcelain pipes which are thus used are furnished only in certain lengths and in designing a system for handling acids it requires that the system be designed with special reference to the pipes and other material which may be obtained, rather than designing the system from the viewpoint of producing its most advantageous arrangement.

The alloy which is herein proposed is easily machinable, that is to say, threads may be cut in the metal, pipe may be cut into different lengths, and in general the alloy may be fabricated and machined the same as iron. In other words, the alloy may be used to make pipes, receptacles, valves, pumps, cocks, etc.

The proposed alloy consists principally of iron, chromium and carbon in the proportion of 40 per cent. of chromium, 58 per cent. to 59 per cent. of iron, and 1 to 2 per cent. of carbon, the carbon existing in the alloy in combined form probably as a carbid of iron and chromium, this carbid

being, so to speak, dissolved in the alloy of 55 chromium and iron.

To this alloy there may be added a small percentage of manganese, which tends to maintain the carbon in the carbid form and to overcome any tendency of the carbon to 60 pass into the graphitic stage when the alloy is cooled from its molten state.

The properties of the alloy are very much enhanced by adding to the iron and chromium a small amount of molybdenum. The 65 amount of molybdenum thus added may vary from 4 to 6 per cent.

Having described my invention, I claim—

1. An acid resisting alloy containing approximately 40 per cent. of chromium, a 70 metal having the properties of molybdenum, together with iron and carbon.

2. An acid resisting alloy containing approximately 40 per cent. of chromium, approximately 4 to 6 per cent. of a metal having the properties of molybdenum, together with iron and carbon.

3. An acid resisting alloy containing approximately 40 per cent. of chromium, a metal having the properties of molybdenum, 80 together with iron and carbid of iron and chromium.

4. An acid resisting alloy containing approximately 40 per cent. of chromium, a metal having the properties of molybdenum, 85 together with iron and 1 to 2 per cent. of carbon.

5. An acid resisting alloy comprising substantially 40 per cent. of chromium, substantially 1 to 2 per cent. of carbon, substantially 4 to 6 per cent. of molybdenum and the remainder of iron.

6. An acid resisting alloy comprising substantially 40 per cent. of chromium, substantially 1½ per cent. of carbon, substantially 4 per cent. of molybdenum and the remainder of iron.

7. An acid resisting alloy containing as principal ingredients iron in excess of 50%, chromium and a metal having the properties of molybdenum.

8. An acid resisting alloy containing as principal ingredients iron in excess of 50%, chromium, and 4 to 6% of a metal having the properties of molybdenum.

In testimony whereof, I hereunto affix my signature.

ALVAH W. CLEMENT.